



US005824176A

# United States Patent [19]

Stein et al.

[11] Patent Number: 5,824,176

[45] Date of Patent: Oct. 20, 1998

## [54] HEAT-TRANSFER LABEL

[75] Inventors: **Samuel H. Stein**, Westborough; **Eleanor R. Snay**, Worcester; **Friedrich H. H. Geurtsen**, Holliston; **James S. Nugent**, Hudson, all of Mass.

[73] Assignee: **Avery Dennison Corporation**, Pasadena, Calif.

[21] Appl. No.: 673,128

[22] Filed: Jul. 1, 1996

[51] Int. Cl.<sup>6</sup> B44C 1/16; B32B 7/06; B32B 27/08

[52] U.S. Cl. 156/239; 156/240; 156/289; 428/200; 428/202; 428/347; 428/349; 428/352; 428/355 R; 428/914

[58] Field of Search 156/239, 240, 156/289; 428/200, 201, 202, 203, 205, 346, 347, 348, 349, 352, 355 R, 914

## [56] References Cited

## U.S. PATENT DOCUMENTS

- 3,907,974 9/1975 Smith .  
 3,922,435 11/1975 Asnes .  
 4,321,185 3/1982 Benitez .  
 4,426,422 1/1984 Daniels .  
 4,536,434 8/1985 Magnotta ..... 156/230 X  
 4,548,857 10/1985 Galante .  
 4,555,436 11/1985 Geurtsen et al. ..... 156/240 X  
 4,662,965 5/1987 DiFrank et al. ..... 156/215  
 4,927,709 5/1990 Parker et al. .  
 4,935,300 6/1990 Parker et al. .  
 4,971,644 11/1990 Mahn, Sr. et al. ..... 156/253

## OTHER PUBLICATIONS

Technical literature, UCAR® phenoxy resins, Union Carbide Corporation, Hackensack, NJ, publicly available before the filing of the present application.

Technical literature, VITEL® 2300 and 2700 polyester resins, Shell Chemical Company, Akron, OH, publicly available before the filing of the present application.

Technical literature, JONBOND® 751 acrylic emulsion, S.C. Johnson & Son, Inc., Racine, WI, publicly available before present appln. filed.

Technical literature, Rhoplex® GL-618 acrylic emulsion, Rohm and Haas, Philadelphia, PA, publicly available before the filing of the present application.

Technical literature, Sequabond® VS 9010 emulsion, Sequa Chemicals, Inc., Chester, South Carolina, publicly available before the filing of the present application.

Technical literature, Joncetyl® 77 acrylic emulsion, S.C. Johnson & Son, Inc., Racine, WI, publicly available before present appln. filed.

Technical literature, Surfynol® 104 surfactant, Air Products, Pittsburgh, PA, publicly available before the filing of the present application.

Technical literature, Triton® X114 surfactant, Union Carbide Corp., Danbury, CT, publicly available before the filing date of the present application.

Primary Examiner—Curtis Mayes  
 Attorney, Agent, or Firm—Kriegsman & Kriegsman

## [57] ABSTRACT

A composition for use in forming an adhesive layer and a heat-transfer label including such an adhesive layer. In one embodiment, the label is designed for use on silane-treated glass containers of the type that are subjected to pasteurization conditions. The label includes a support portion and a transfer portion, the transfer portion being positioned over the support portion. The support portion includes a sheet of paper overcoated with a release layer of polyethylene. The transfer portion includes an organic solvent-soluble phenoxy protective lacquer layer, an organic solvent-soluble polyester ink layer over the protective lacquer layer, and an acrylic adhesive layer over the ink layer. The adhesive layer is formed by depositing onto the ink layer, e.g., by gravure printing, a composition comprising a water-based acrylic resin dispersion or emulsion, isopropyl alcohol and water, and then evaporating the volatile components of the composition to leave an acrylic film.

17 Claims, 1 Drawing Sheet





FIG. 1



FIG. 2

## HEAT-TRANSFER LABEL

## BACKGROUND OF THE INVENTION

The present invention relates generally to heat-transfer labels and more particularly to heat-transfer labels of the type having an adhesive layer for adhering the label to a desired article.

Heat-transfer labels are commonly used in the decorating and/or labelling of commercial articles, such as, and without limitation to, containers for beverages (including alcoholic beverages such as beer), essential oils, detergents, adverse chemicals, as well as health and beauty aids. As can readily be appreciated, heat-transfer labels are desirably resistant to abrasion and chemical effects in order to avoid a loss of label information and desirably possess good adhesion to the articles to which they are affixed.

One well-known type of heat-transfer label is described in U.S. Pat. No. 3,616,015, inventor Kingston, which issued October, 1971, and which is incorporated herein by reference. In the aforementioned patent, there is disclosed a heat-transfer label comprising a paper sheet or web, a wax release layer affixed to the paper sheet, and an ink design layer printed on the wax release layer. In the heat-transfer labelling process, the label-carrying web is subjected to heat, and the label is pressed onto an article with the ink design layer making direct contact with the article. As the paper sheet is subjected to heat, the wax layer begins to melt so that the paper sheet can be released from the wax layer. After transfer of the design to the article, the paper sheet is immediately removed, leaving the design firmly affixed to the article and the wax layer exposed to the environment. The wax layer is thus intended to serve two purposes: (1) to provide release of the ink design from the web upon application of heat to the web and (2) to form a protective layer over the transferred ink design. After transfer of the label to the article, the transferred wax release layer is typically subjected to a post-flaming technique which enhances the optical clarity of the wax protective layer (thereby enabling the ink design layer therebeneath to be better observed) and which enhances the protective properties of the transferred wax release.

In some heat-transfer labels, an adhesive layer (e.g., solvent-soluble polyamide, acrylic or polyester) is deposited over the ink design to facilitate adhesion of the label onto a receiving article. An example of a heat-transfer label having an adhesive layer is disclosed in U.S. Pat. No. 4,548,857, inventor Galante, which issued Oct. 22, 1985, and which is incorporated herein by reference. Additionally, in some heat-transfer labels, a protective lacquer layer is interposed between the wax release layer and the ink layer. An example of such a label is disclosed in U.S. Pat. No. 4,426,422, inventor Daniels, which issued Jan. 17, 1984, and which is incorporated herein by reference.

One problem that has been noted with heat-transfer labels of the type described above containing a wax release layer is that, quite often, a degree of hazing or a "halo" is noticeable over the transferred label when the transfer is made onto clear materials. This "halo" effect, which persists despite post-flaming, is a result of the nature of the wax coating around the outer borders of the transferred ink design layer. Hazing due to the wax release layer may also appear in "open-copy" areas of the label, i.e., areas of the label where no ink is present between the adhesive and protective lacquer layers, and also represents a problem.

Accordingly, to overcome the aforementioned "halo" effect, considerable effort has been expended in replacing or

obviating the need for a wax release layer. One such wax-less, heat-transfer label is disclosed in U.S. Pat. No. 3,922,435, inventor Asnes, which issued Nov. 25, 1975. In the aforementioned patent, the layer of wax is replaced with a layer of a non-wax resin. This non-wax resinous layer is referred to in the patent as a dry release since it does not transfer to the article along with the ink design layer. In a preferred embodiment of the patent, the non-wax resinous layer comprises a thermoset polymeric resin, such as cross-linked resins selected from the group consisting of acrylic resins, polyamide resins, polyester resins, vinyl resins and epoxy resins.

Another example of a wax-less, heat-transfer label is disclosed in U.S. Pat. No. 4,935,300, inventors Parker et al., which issued Jun. 19, 1990, and which is incorporated herein by reference. In the aforementioned patent, the label, which is said to be particularly well-suited for use on high density polyethylene, polypropylene, polystyrene, polyvinylchloride and polyethylene terephthalate surfaces or containers, comprises a paper carrier web which is overcoated with a layer of polyethylene. A protective lacquer layer comprising a polyester resin and a relatively small amount of a non-drying oil is printed onto the polyethylene layer. An ink design layer comprising a resinous binder base selected from the group consisting of polyvinylchloride, acrylics, polyamides and nitrocellulose is then printed onto the protective lacquer layer. A heat-activatable adhesive layer comprising a thermoplastic polyamide adhesive is then printed onto the ink design layer.

Although the above-described wax-less, heat-transfer label eliminates the wax-related "halo" effect discussed previously, said label does not quite possess the same release characteristics of heat-transfer labels containing a wax release layer. Accordingly, another type of heat-transfer label differs from the heat-transfer label disclosed in U.S. Pat. No. 4,935,300, only in that a very thin layer or "skim coat" of a waxlike material is interposed between the polyethylene release layer and the protective lacquer layer to improve the release of the protective lacquer from the polyethylene-coated carrier web. The thickness of the skim coat corresponds to approximately 0.1-0.4 lbs. of the waxlike material spread onto about 3000 square feet of the polyethylene release layer.

The aforementioned type of heat-transfer label may be used to decorate a variety of surfaces and materials including glass containers. Glass containers are frequently, although not invariably, pre-treated (typically by the container manufacturer) with polyethylene, oleic acid, stearate or a similar material whose function is to enhance abrasion resistance and lubricity. Such containers, whether or not previously subjected to the foregoing type of pre-treatment (or whether or not such a pre-treatment is later removed from the container), are typically treated, prior to decoration, with a silane adhesion promoter of the type described in U.S. Pat. No. 3,907,974, inventor Smith, which issued Sep. 23, 1975 and which is incorporated herein by reference. An example of a heat-transfer label used by the assignee of the present application to label silane-treated glass containers comprises a paper carrier web overcoated with a layer of polyethylene. A skim coat is overcoated on the polyethylene layer, and a phenoxy lacquer layer is printed on the skim coat. A polyester ink design layer is printed on the lacquer layer, and a solvent-soluble polyester adhesive layer is printed on the ink design layer.

Although the aforementioned heat-transfer label generally adheres well and looks good when applied to glass containers, it has been noted that, when said labelled glass

containers are subjected to the heat and moisture conditions of pasteurization (as is the case, for example, where the labelled containers are filled with beer and the beer is pasteurized while in the glass container), the pasteurization process often gives the label a hazy appearance (particularly in open-copy areas), presumably caused by penetration of water into the label during pasteurization. Some amelioration of the haze may be achieved by heating the label to remove water therefrom; however, as can readily be appreciated, this approach may be impractical in many instances.

Another problem that has been noted in connection with existing heat-transfer labels is that heat-transfer labels of the type described above simply do not adhere well to many commercially-available aluminum cans due to a highly-lubricating acrylic coating or varnish that is typically applied to the cans during manufacturing to make them more resistant to scratching, abrasion and the like. White inks are also frequently used in combination with such varnishes as pre-treatment coatings on aluminum cans and similarly pose an adhesion problem for labels. Aluminum cans are not treated with an adhesion promoter comparable to the silane promoter used on glass containers.

#### SUMMARY OF THE INVENTION

It is an object of the present invention to provide a novel heat-transfer label.

It is another object of the present invention to provide a heat-transfer label as described above that overcomes at least some of the problems discussed above in connection with existing heat-transfer labels.

It is still another object of the present invention to provide a novel adhesive layer for use in a heat-transfer label.

In furtherance of the above and other objects that are herein disclosed or are apparent from the present specification, there is provided a heat-transfer label which comprises (a) a support portion; and (b) a transfer portion over said support portion for transfer of the transfer portion from the support portion to an article upon application of heat to the support portion while the transfer portion is placed into contact with the article, said transfer portion comprising (i) a protective lacquer layer; (ii) an ink layer over said protective lacquer layer; and (iii) an adhesive layer over said ink layer, said adhesive layer comprising an adhesive of the type present in a water-based adhesive emulsion or in a water-based adhesive dispersion.

According to a first embodiment of the invention, the heat-transfer label is particularly well-suited for use on silane-treated glass containers of the type that are subjected to pasteurization conditions (regardless of whether the glass containers have previously been pre-treated with polyethylene, oleic acid, stearate or the like), said heat-transfer label comprising (a) a support portion comprising a sheet of paper overcoated with a release layer of polyethylene; and (b) a transfer portion over said support portion for transfer of the transfer portion from the support portion to an article upon application of heat to the support portion while the transfer portion is placed into contact with the article, said transfer portion comprising (i) a protective lacquer layer; (ii) an ink layer over said protective lacquer layer; and (iii) an adhesive layer over said ink layer, said adhesive layer comprising an adhesive of the type present in a water-based adhesive emulsion or in a water-based adhesive dispersion.

Preferably, the protective lacquer layer comprises a phenoxy lacquer, a polyester lacquer, a polyester/vinyl lacquer or an acrylic lacquer, and the ink layer comprises a polyester

ink, a polyester/vinyl ink, a polyamide ink or an acrylic ink. The adhesive layer of the aforementioned heat-transfer label is preferably formed by (a) depositing onto the ink layer, for example by gravure printing or the like, a layer of a composition comprising (i) a water-based all-acrylic thermoplastic polymer emulsion and (ii) a surface tension lowering agent; and (b) evaporating the volatile components of the composition.

The adhesive composition may comprise, for example, (i) a water-based all-acrylic thermoplastic polymer emulsion having a solids content of approximately 46.5-47.5%, by weight, a pH of about 7.5-9.5, a specific gravity of about 1.07 at 25° C., a weight of about 8.9 pounds/U.S. gallon, a Brookfield LVF Viscosity at 30 rpm, #2 spindle, of about 300-500 cps, a minimum film formation temperature of about 20° C. and a glass transition temperature of about 27° C., said water-based all-acrylic thermoplastic polymer emulsion constituting about 74.5%, by weight, of said adhesive composition, (ii) isopropyl alcohol in an amount constituting about 17.5%, by weight, of said adhesive composition, and (iii) water in an amount constituting about 7.5%, by weight, of said adhesive composition.

According to a second embodiment of the invention, the heat-transfer label is particularly well-suited for use on aluminum cans of the type that have been treated with a highly-lubricating acrylic coating or varnish of the type used to prevent scratching and abrasion of such cans (said varnish either being used alone or in combination with a white ink), said heat-transfer label comprising (a) a support portion comprising a sheet of paper overcoated with a release layer of polyethylene; and (b) a transfer portion over said support portion for transfer of the transfer portion from the support portion to an article upon application of heat to the support portion while the transfer portion is placed into contact with the article, said transfer portion comprising (i) a protective lacquer layer; (ii) an ink layer over said protective lacquer layer; and (iii) an adhesive layer over said ink layer, said adhesive layer comprising an adhesive of the type present in a water-based adhesive emulsion or in a water-based adhesive dispersion.

Preferably, the protective lacquer layer comprises an acrylic lacquer, a phenoxy lacquer, a polyester/vinyl lacquer or a polyester lacquer, and the ink layer comprises a polyester ink, a polyester/vinyl ink, a polyamide ink or an acrylic ink. The adhesive layer of the aforementioned heat-transfer label is preferably formed by (a) depositing onto the ink layer, for example by gravure printing or the like, a layer of a composition comprising (i) a water-based acrylic polymer emulsion and (ii) a surface tension lowering agent; and (b) evaporating the volatile components of the composition.

The adhesive composition may comprise, for example, (i) an acrylic polymer emulsion having a solids content of approximately 45%, by weight, a pH of about 8.3, a weight of about 8.7 pounds/U.S. gallon, a Brookfield viscosity of about 450 cps and a glass transition temperature of about 21° C., said acrylic polymer emulsion constituting about 80%, by weight, of said adhesive composition, (ii) isopropyl alcohol in an amount constituting about 14%, by weight, of said adhesive composition, and (iii) water in an amount constituting about 6%, by weight, of said adhesive composition.

In addition to being directed to the above-described heat-transfer labels, the present invention is also directed to the transfer portion of the heat-transfer labels, as well as to the adhesive compositions used to form the adhesive layers of the heat-transfer labels, to methods for forming the

adhesive layers with the aforementioned adhesive compositions, to the adhesive layers formed using the foregoing adhesive compositions, and to methods of labelling surfaces with the above-described heat-transfer labels.

For purposes of the present specification and claims, it is to be understood that certain terms used herein, such as "on" or "over," when used to denote the relative positions of two or more layers of a heat-transfer label, are primarily used to denote such relative positions in the context of how those layers are situated prior to transfer of the transfer portion of the label to an article since, after transfer, the arrangement of layers is inverted as those layers which were furthest removed from the associated support sheet are now closest to the labelled article.

Additional objects, as well as features, advantages and aspects of the present invention, will be set forth in part in the description which follows, and in part will be obvious from the description or may be learned by practice of the invention. In the description, reference is made to the accompanying figures which form a part thereof and in which is shown by way of illustration specific embodiments for practicing the invention. These embodiments will be described in sufficient detail to enable those skilled in the art to practice the invention, and it is to be understood that other embodiments may be utilized and that structural changes may be made without departing from the scope of the invention. The following detailed description is, therefore, not to be taken in a limiting sense, and the scope of the present invention is best defined by the appended claims.

#### BRIEF DESCRIPTION OF THE DRAWINGS

The accompanying figures, which are hereby incorporated into and constitute a part of this specification, illustrate preferred embodiments of the invention and, together with the description, serve to explain the principles of the invention. In the figures wherein like reference numerals represent like parts:

FIG. 1 is a schematic section view of a first embodiment of a heat-transfer label that is particularly well-suited for, but not limited to, use on silane-treated glass containers of the type that are subjected to pasteurization conditions, the heat-transfer label being constructed according to the teachings of the present invention; and

FIG. 2 is a schematic section view of a second embodiment of a heat-transfer label that is particularly well-suited for, but not limited to, use on aluminum cans of the type that have been treated with a highly-lubricating thermoset acrylic coating used to prevent scratching and abrasion of such cans, the heat-transfer label being constructed according to the teachings of the present invention.

#### DETAILED DESCRIPTION OF PREFERRED EMBODIMENTS

Referring now to FIG. 1, there is shown a schematic section view of a first embodiment of a heat-transfer label that is particularly well-suited for, but not limited to, use on silane-treated glass containers of the type that are subjected to pasteurization conditions (e.g., silane-treated glass containers used to hold pasteurized beer, the beer being pasteurized while in the glass containers), the heat-transfer label being constructed according to the teachings of the present invention and being represented generally by reference numeral 11. (It is to be understood that, for purposes of the present specification and claims, the expression "silane-treated glass containers" refers both to silane-treated glass containers that have been pre-treated with an abrasion-

resistance material, such as polyethylene, oleic acid, stearate or the like, and to silane-treated glass containers that have not been so pre-treated.)

Label 11 comprises a support portion 13. Support portion 13, in turn, comprises a carrier web 15 overcoated with a polyethylene layer 17. Carrier web 15 is typically made of paper or a similarly suitable substrate. Details of polyethylene layer 17 are disclosed in U.S. Pat. No. 4,935,300, discussed above, and in U.S. Pat. No. 4,927,709, inventors Parker et al., which issued on May 22, 1990, which is incorporated herein by reference.

Label 11 also comprises a skim coat 19 of the type described above, which is coated directly on top of the entirety of polyethylene layer 17. During label transfer, a small portion of skim coat 19 may be transferred along with the transfer portion of label 11 onto the article being labelled, the amount of skim coat 19 transferred onto the article being labelled not being readily discernible.

Label 11 further comprises a transfer portion 21. Transfer portion 21, in turn, includes a protective lacquer layer 23 printed directly on top of a portion of skim coat 19, an ink design layer 25 printed onto a desired area of lacquer layer 23, and a heat-activatable adhesive layer 27 printed onto design layer 25.

Protective lacquer layer 23 comprises a phenoxy lacquer resin, a polyester lacquer resin, a polyester/vinyl lacquer resin and/or an acrylic lacquer resin. Examples of phenoxy lacquer resins include the UCAR® Phenoxy Resins (Union Carbide Corporation, Hackensack, N.J.), which have the following chemical structure:



A particularly preferred UCAR® Phenoxy Resin is PKHH, a medium weight grade of the above structure which, at 40% solids, by weight, in methyl ethyl ketone (MEK), has a solution viscosity of 4500 to 7000 mPa·s(cP). To form lacquer layer 23, a lacquer composition comprising a lacquer resin and one or more suitable volatile solvents are deposited onto a desired area of skim coat 19, preferably by gravure printing or a similar technique. After deposition of the lacquer composition onto the desired area of skim coat 19, the volatile solvent(s) evaporate(s), leaving only the non-volatile components thereof to make up lacquer layer 23. Where the lacquer resin is PKHH, the lacquer composition preferably comprises about 25%, by weight, PKHH; about 46.6%, by weight, methyl ethyl ketone; about 23.4%, by weight, toluene; and about 5.0%, by weight, Dowanol PM propylene glycol methyl ether (Dow Chemical).

Ink design layer 25 of transfer portion 21 comprises a polyester/vinyl ink, a polyamide ink, an acrylic ink and/or a polyester ink. Ink design layer 25 is formed in the conventional manner by depositing, by gravure printing or the like, an ink composition comprising a resin of the type described above, a suitable pigment or dye and one or more suitable volatile solvents onto one or more desired areas of lacquer layer 23. After application of the ink composition onto lacquer layer 23, the volatile solvent component(s) of the ink solvent system evaporate(s), leaving only the non-volatile ink components to form layer 25. An example of a suitable resin for use in forming a polyester ink is ViTEL® 2700 (Shell Chemical Company, Akron, Ohio)—a copolyester resin having a high tensile strength (7000 psi) and a low

elongation (4% elongation). A ViTEL® 2700-based polyester ink composition may comprise, by weight, 18% ViTEL® 2700, 6% pigment, 30.4% n-propyl acetate (NP Ac) and 45.6% toluene. As can readily be appreciated, ViTEL® 2700 is, by no means, the only polyester resin that may be used to formulate a polyester ink, and solvent systems, other than an NP Ac:toluene system, may be suitable for use with ViTEL® 2700, as well as with other polyester resins.

Adhesive layer 27 of transfer portion 21 comprises an acrylic adhesive of the type present in a water-based adhesive emulsion or a water-based adhesive dispersion (as contrasted with a water-soluble or an organic solvent-soluble acrylic adhesive). Adhesive layer 27 is formed by depositing onto ink layer 25, by gravure printing or the like, an adhesive composition comprising a water-based acrylic adhesive emulsion or dispersion and a surface tension lowering agent. After application of the adhesive composition onto ink layer 25, the volatile components of the composition (e.g., water, alcohol) evaporate, leaving only the non-volatile solid components thereof to form layer 27.

Examples of the water-based acrylic emulsion include RHOPLEX® GL-618 emulsion (Rohm and Haas, Philadelphia, Pa.)—a water-based all-acrylic elastomeric polymer emulsion having a solids content of approximately 46.5–47.5%, by weight, a pH of about 7.5–9.5, a specific gravity of about 1.07 at 25° C., a weight of about 8.9 pounds/U.S. gallon, a Brookfield LVF Viscosity at 30 rpm, #2 spindle, of about 300–500 cps, a minimum film formation temperature of about 20° C. and a glass transition temperature of about 27° C.; JONCRYL 77 (S.C. Johnson & Son, Inc., Racine, Wis.)—an acrylic polymer emulsion having a solids content of approximately 45%, by weight, a pH of about 8.3, a weight of about 8.7 pounds/U.S. gallon, a Brookfield viscosity of about 450 cps and a glass transition temperature of about 21° C.; JONBOND® 751 (S.C. Johnson & Son, Inc., Racine, Wis.)—an acrylic emulsion having a solids content of approximately 46±1%, by weight, a pH of about 7.4–7.8, a weight of about 8.7 pounds/gallon, a Brookfield LVF viscosity of 700±200 cps and an activation temperature of approximately 93.3° C.; and SEQUABOND® VS 9010 (Sequa Chemicals, Inc., Chester, S.C.)—a polymer emulsion having a solids content of approximately 47%, a pH of about 8.5, a viscosity of about 600 cps, a weight of about 8.7 pounds/gallon and a glass transition temperature of about –30° C.

The purpose of the above-identified surface tension lowering agent is to reduce the surface tension of the water-based adhesive emulsion or dispersion sufficiently to enable the composition to be deposited (e.g., printed) onto ink layer 25 in the form of a substantially continuous film for good printing quality—in other words, to prevent the composition from striating or yielding poor printing quality when deposited on top of ink layer 25 during printing. Suitable surface tension lowering agents include, but are not limited to, (i) alcohols that are efficient at lowering surface tension and (ii) relatively hydrophobic, low-foaming, asymmetrical surfactants of low molecular weight. Examples of surface tension lowering agents include isopropyl alcohol, n-propyl alcohol, polypropylene oxide-ethylene oxide-polypropylene oxide and 2,4,7,9-tetramethyl-5-decyne-4,7-diol (commercially available from Air Products, Pittsburgh, Pa. as Surfynol® 104 surfactant). It should be noted, however, that the amount of alcohol in the composition is small compared to the amount of water in the composition as the alcohol is not used to put the resin into solution.

In addition to reducing surface tension, the above-described surface tension lowering agent, as well as the

additional water added to the emulsion and surface tension lowering agent, also serves to lower the yield value (i.e., rheology) of the composition to facilitate printing of the composition.

5 The following are illustrative examples of adhesive compositions that may be used to form adhesive layer 27, it being understood that other adhesive compositions of the general type described above may also be used to form adhesive layer 27 and that the examples given below are in 10 no way intended to be limiting:

#### EXAMPLE 1

|                                    |                     |
|------------------------------------|---------------------|
| RHOPLEX® GL-618 emulsion           | approximately 74.5% |
| Isopropyl alcohol                  | approximately 17.4% |
| Water                              | approximately 7.4%  |
| Water soluble fluorescent material | approximately 0.6%  |

20 Mix together the isopropyl alcohol and water. While stirring the acrylic emulsion, add the alcohol/water mixture thereto. Then, add the fluorescent material (which is added to the formulation merely for registration purposes during printing.) The surface tension of the formulation is about 28 25 dynes/cm.

#### EXAMPLE 2

|                                    |                   |
|------------------------------------|-------------------|
| JONCRYL 77 emulsion                | approximately 83% |
| Water                              | approximately 17% |
| Water soluble fluorescent material | <1%               |

#### EXAMPLE 3

|                                    |                     |
|------------------------------------|---------------------|
| JONCRYL 77 emulsion                | approximately 62.1% |
| RHOPLEX® GL-618 emulsion           | approximately 20.8% |
| Isopropyl alcohol                  | approximately 11.4% |
| Water                              | approximately 4.9%  |
| Water soluble fluorescent material | approximately 0.6%  |

#### EXAMPLE 4

|                                    |                   |
|------------------------------------|-------------------|
| Joncryl 77 emulsion                | approximately 80% |
| Isopropyl alcohol                  | approximately 14% |
| Water                              | approximately 6%  |
| Water soluble fluorescent material | <1%               |

50 Mix together the isopropyl alcohol and water. While stirring the acrylic emulsion, add the alcohol/water mixture thereto. Then, add the fluorescent material.

#### EXAMPLE 5

|                                    |                     |
|------------------------------------|---------------------|
| Sequabond® VS 9010                 | approximately 79.5% |
| Isopropyl alcohol                  | approximately 13.9% |
| Water                              | approximately 5.9%  |
| Water soluble fluorescent material | approximately 0.6%  |

65 Mix together the isopropyl alcohol and water. While stirring the acrylic emulsion, add the alcohol/water mixture thereto. Then, add the fluorescent material.

## EXAMPLE 6

|                                    |                     |
|------------------------------------|---------------------|
| RHOPLEX® GL-618 emulsion           | approximately 87.5% |
| n-propyl alcohol                   | approximately 10.2% |
| Water                              | approximately 1.4%  |
| Water soluble fluorescent material | approximately 0.7%  |

While the acrylic emulsion is under agitation, add the n-propyl alcohol thereto. Next, add the water to the mixture. Then, add the fluorescent material to the mixture.

## EXAMPLE 7

|                                                               |                     |
|---------------------------------------------------------------|---------------------|
| RHOPLEX® GL-618 emulsion                                      | approximately 73.4% |
| Isopropyl alcohol                                             | approximately 17.1% |
| Water                                                         | approximately 7.3%  |
| Triton® X114 nonionic surfactant (Union Carbide, Danbury, CT) | approximately 1.5%  |
| Water soluble fluorescent material                            | approximately 0.6%  |

Mix together the isopropyl alcohol, Triton® X114 and water. While stirring the acrylic emulsion, add the alcohol/Triton® X114/water mixture thereto. Then, add the fluorescent material.

## EXAMPLE 8

|                                    |                     |
|------------------------------------|---------------------|
| JONBOND® 751 emulsion              | approximately 84.5% |
| n-propyl alcohol                   | approximately 14.8% |
| Water soluble fluorescent material | approximately 0.6%  |

While the acrylic emulsion is under agitation, add the n-propyl alcohol thereto. Then, add the fluorescent material to the mixture.

## EXAMPLE 9

|                                    |                     |
|------------------------------------|---------------------|
| JONCRYL 77 emulsion                | approximately 59.6% |
| JONBOND® 751 emulsion              | approximately 19.9% |
| Isopropyl alcohol                  | approximately 13.9% |
| Water                              | approximately 5.9%  |
| Water soluble fluorescent material | approximately 0.6%  |

Mix together the isopropyl alcohol and water. While stirring together the two acrylic emulsions, add the alcohol/water mixture thereto. Then, add the fluorescent material.

## EXAMPLE 10

|                                                             |                     |
|-------------------------------------------------------------|---------------------|
| JONCRYL 77 emulsion                                         | approximately 77.6% |
| Surfynol® 104PA (50% wt Surfynol® 104 in isopropyl alcohol) | approximately 4.4%  |
| Isopropyl alcohol                                           | approximately 11.6% |
| Water                                                       | approximately 5.8%  |
| Water soluble fluorescent material                          | approximately 0.6%  |

Mix together the isopropyl alcohol and water. While stirring together the acrylic emulsion, add the alcohol/water mixture thereto. Next, add the Surfynol® 104PA. Then, add the fluorescent material.

5

## EXAMPLE 11

|                                    |                     |
|------------------------------------|---------------------|
| JONCRYL 77 emulsion                | approximately 19.9% |
| JONBOND® 751 emulsion              | approximately 59.6% |
| Isopropyl alcohol                  | approximately 13.9% |
| Water                              | approximately 5.9%  |
| Water soluble fluorescent material | approximately 0.6%  |

10 Mix together the isopropyl alcohol and water. While stirring together the two acrylic emulsions, add the alcohol/water mixture thereto. Then, add the fluorescent material.

## EXAMPLE 12

|                                                            |                     |
|------------------------------------------------------------|---------------------|
| JONCRYL 77 emulsion                                        | approximately 84.1% |
| Surfynol® 104NP (50% wt Surfynol® 104 in n-propyl alcohol) | approximately 10.5% |
| Water                                                      | approximately 4.7%  |
| Water soluble fluorescent material                         | approximately 0.6%  |

20

While stirring the emulsion, add the water thereto. Next, add the Surfynol® 104NP. Then, add the fluorescent material.

25 Label 11 may be used in the conventional manner by contacting adhesive layer 27 to a desired article, such as a glass container, while applying sufficient heat to the bottom of carrier web 15 so as to cause transfer portion 21 to be released from support portion 13 and so as to cause adhesive layer 27 to become heat-activated for bonding to the desired article.

30 The present inventors have noted that, when label 11 is applied to silane-treated glass containers and said labelled containers are subsequently subjected to pasteurization conditions, the above-mentioned problem of open-copy hazing is substantially ameliorated (with best results being observed when the adhesive compositions of Examples 1 and 4-12 are used to form adhesive layer 27). The present inventors have also noted that label 11 (employing a phenoxy lacquer 23, a polyester ink layer 25 and an adhesive layer of any of Examples 1-12) adheres well to silane-treated glass containers and that the constituent layers of label 11 possess excellent interlayer adhesion (as observed in tape tests, i.e., tests which involve applying a piece of adhesive tape to a label on an article, removing the piece of tape and checking the integrity of the label.) Moreover,

35 40 45 50 55 adhesive composition is an emulsion, as opposed to a solution, higher molecular weight resins possessing better adhesion may be used in the present emulsion than could be used in comparable solutions (due to viscosity constraints on printing with such solutions)—thereby leading to improved adhesion properties between the label and the container. Furthermore, the present inventors have noted that label 11 possesses a high degree of abrasion resistance.

55 Referring now to FIG. 2, there is shown a schematic section view of a second embodiment of a heat-transfer label that is particularly well-suited for, but not limited to, use on aluminum cans of the type that have been treated with a highly-lubricating acrylic coating or varnish used to prevent scratching and abrasion of such cans (and which may or may not have also been treated with a white ink), the heat-transfer label being constructed according to the teachings of the present invention and being represented generally by reference numeral 111.

60 65 65 Label 111 comprises a support portion 113. Support portion 113 is identical to support portion 13 of label 11 and

## 11

comprises a carrier web 115 overcoated with a polyethylene layer 117. Label 111 also comprises a skim coat 119 which is identical to skim coat 19 of label 11.

Label 111 further comprises a transfer portion 121. Transfer portion 121, in turn, includes a protective lacquer layer 123 printed directly on top of a portion of skim coat 119, an ink design layer 125 printed onto a desired area of lacquer layer 123, and a heat-activatable adhesive layer 127 printed onto design layer 125.

Protective lacquer layer 123, like protective lacquer layer 23 of label 11, comprises an acrylic lacquer resin, a phenoxy lacquer resin, a polyester/vinyl lacquer resin and/or a polyester lacquer resin. To form lacquer layer 123, a lacquer composition comprising one or more lacquer resins and one or more suitable volatile solvents are deposited onto a desired area of skim coat 119, preferably by gravure printing or a similar technique. After deposition of the lacquer composition on the desired area of skim coat 119, the volatile solvent(s) evaporate(s), leaving only the non-volatile components thereof to make up lacquer layer 123. A particularly preferred lacquer layer 123 comprises a combination of ELVACITE® 2013 acrylic resin (ICI Acrylics Inc., Wilmington, Del.), a low molecular weight methyl/n-butyl methacrylate copolymer having an inherent viscosity of 0.17 (as measured in a solution containing 0.25 g of polymer in 50 ml methylene chloride, measured at 20° C. using a No. 50 Cannon-Fenske Viscometer), and ELVACITE® 2014 acrylic resin (ICI Acrylics Inc., Wilmington, Del.), a medium molecular weight methyl methacrylate copolymer having an inherent viscosity of 0.40 (as measured in the manner described above).

Ink design layer 125 of transfer portion 121, like ink design layer 25 of label 11, comprises an acrylic ink, a polyester ink, a polyester/vinyl ink and/or a polyamide ink. Ink design layer 125 is formed in the conventional manner by depositing, by gravure printing or the like, an ink composition comprising the ink(s) and one or more suitable volatile solvents onto one or more desired areas of lacquer layer 123. After application of the ink composition onto lacquer layer 123, the volatile solvent component of the ink composition evaporates, leaving only the non-volatile ink component to form layer 125. A particularly preferred type of ink for ink design layer 125 are acrylic inks.

Adhesive layer 127 of transfer portion 121, like adhesive layer 27 of label 11, comprises an acrylic adhesive of the type present in a water-based adhesive emulsion or dispersion. Adhesive layer 127 is formed by depositing onto ink layer 125, by gravure printing or the like, an adhesive composition comprising a water-based acrylic adhesive emulsion or dispersion and a surface tension lowering agent. Suitable adhesive compositions useful in forming adhesive layer 127 include the adhesive compositions of Examples 2 through 5 and 8 through 12 above, with the adhesive compositions of Examples 4 and 12 being preferred. After application of the adhesive composition onto ink layer 125, the volatile components of the composition (i.e., water, certain alcohols) evaporate, leaving only the non-volatile solid components thereof (i.e., resin, certain surfactants) to form layer 127.

Label 111 may be used in the conventional manner by contacting adhesive layer 127 to a desired article while applying sufficient heat to the bottom of carrier web 115 so as to cause transfer portion 121 to be released from support portion 113 and so as to cause adhesive layer 127 to become heat-activated for bonding to the desired article.

Using the above-described tape tests, the present inventors have noted that, when label 111 is applied to aluminum

## 12

cans of the type described above, excellent adhesion is achieved between label 111 and the aluminum can. In addition, the present inventors have noted that label 111 exhibits excellent interlayer adhesion of its constituent layers and that label 111 possesses excellent abrasion resistance.

The embodiments of the present invention recited herein are intended to be merely exemplary and those skilled in the art will be able to make numerous variations and modifications to it without departing from the spirit of the present invention. All such variations and modifications are intended to be within the scope of the present invention as defined by the claims appended hereto.

What is claimed is:

1. A method of labelling an article, the article being a silane-treated glass container, said method comprising the steps of:

(a) providing a heat-transfer label, said heat-transfer label comprising:

(i) a support portion, and  
(ii) a transfer portion over said support portion for transfer of the transfer portion from the support portion to the article upon application of heat to the support portion while the transfer portion is placed into contact with the article, said transfer portion comprising an adhesive layer, said adhesive layer comprising an adhesive of the type present in a water-based adhesive emulsion or in a water-based adhesive dispersion, said adhesive being an acrylic adhesive, the transfer portion further comprising an ink layer and a protective lacquer layer, said protective lacquer layer comprising an organic solvent-soluble phenoxy lacquer, said ink layer being positioned over said protective lacquer layer and comprising an organic solvent-soluble polyester ink, said adhesive layer being positioned over said ink layer; and

(b) transferring said transfer portion from said support portion to the article.

2. A heat-transfer label comprising:

(a) a support portion; and

(b) a transfer portion over said support portion for transfer of the transfer portion from the support portion to an article upon application of heat to the support portion while the transfer portion is placed into contact with the article, said transfer portion comprising:

(i) a protective lacquer layer wherein said protective lacquer layer comprises a phenoxy lacquer;  
(ii) an ink layer over said protective lacquer layer; and  
(iii) an adhesive layer over said ink layer, said adhesive layer comprising an adhesive of the type present in a water-based adhesive emulsion or in a water-based adhesive dispersion.

3. A transfer portion of a heat-transfer label, said transfer portion comprising:

(a) an ink design layer;

(b) an adhesive layer positioned over said ink design layer, said adhesive layer comprising an adhesive of the type present in a water-based adhesive emulsion or in a water-based adhesive dispersion; and

(c) a protective lacquer layer, said ink design layer being positioned over said protective lacquer layer, said protective lacquer layer comprising a phenoxy lacquer.

4. A heat-transfer label comprising:

(a) a support portion; and

(b) a transfer portion over said support portion for transfer of the transfer portion from the support portion to an

**13**

article upon application of heat to the support portion while the transfer portion is placed into contact with the article, said transfer portion comprising:

- (i) a protective lacquer layer wherein said protective lacquer layer comprises a phenoxy lacquer;
- (ii) an ink layer over said protective lacquer layer wherein said ink layer comprises a polyester ink; and
- (iii) an adhesive layer over said ink layer, said adhesive layer comprising an adhesive of the type present in a water-based adhesive emulsion or in a water-based adhesive dispersion.

5. The heat-transfer label as claimed in claim 1 wherein said adhesive of said adhesive layer is an acrylic adhesive.

6. The heat-transfer label as claimed in claim 1 wherein said adhesive layer further comprises a surface tension 15 lowering agent.

7. The heat-transfer label as claimed in claim 6 wherein said surface tension lowering agent is an asymmetric, low molecular weight, hydrophobic, low-foaming surfactant.

8. The heat-transfer label as claimed in claim 7 wherein 20 said surface tension lowering agent is 2,4,7,9-tetramethyl-5-decyne-4,7-diol.

9. The heat-transfer label as claimed in claim 1 wherein said transfer portion is in direct contact with said support portion.

25 10. The heat-transfer label as claimed in claim 1 wherein said support portion comprises a sheet of paper overcoated with a release layer of polyethylene.

11. The heat-transfer label as claimed in claim 4 further comprising a skim coat, said skim coat being interposed 30 between said transfer portion and said support portion.

12. A transfer portion of a heat-transfer label, said transfer portion comprising:

- (a) a protective lacquer layer wherein said protective lacquer layer comprises a phenoxy lacquer;
- (b) an ink design layer positioned over said protective lacquer layer wherein said ink design layer comprises a polyester ink; and
- (c) an adhesive layer positioned over said ink design layer, 35 said adhesive layer comprising an adhesive of the type present in a water-based adhesive emulsion or in a water-based adhesive dispersion.

13. The transfer portion as claimed in claim 12 wherein said adhesive is an acrylic adhesive.

45 14. The transfer portion as claimed in claim 12 wherein said adhesive layer further comprises a surface tension lowering agent.

**14**

15. The transfer portion as claimed in claim 14 wherein said surface tension lowering agent is an asymmetric, low molecular weight, hydrophobic, low-foaming surfactant.

16. A heat-transfer label comprising:

- (a) a support portion; and
  - (b) a transfer portion over said support portion for transfer of the transfer portion from the support portion to an article upon application of heat to the support portion while the transfer portion is placed into contact with the article, said transfer portion comprising:
- (i) a protective lacquer layer;
  - (ii) an ink layer over said protective lacquer layer; and
  - (iii) an adhesive layer over said ink layer, said adhesive layer comprising an adhesive of the type present in a water-based adhesive emulsion or in a water-based adhesive dispersion, said adhesive being the type present in an all-acrylic elastomeric polymer emulsion having a solids content of approximately 46.5–47.5%, by weight, a pH of about 7.5–9.5, a specific gravity of about 1.07 at 25° C., a weight of about 8.9 pounds/U.S. gallon, a Brookfield LVF Viscosity at 30 rpm, #2 spindle, of about 300–500 cps, a minimum film formation temperature of about 20° C. and a glass transition temperature of about 27° C.

17. A heat-transfer label comprising:

- (a) a support portion; and
  - (b) a transfer portion over said support portion for transfer of the transfer portion from the support portion to an article upon application of heat to the support portion while the transfer portion is placed into contact with the article, said transfer portion comprising:
- (i) a protective lacquer layer;
  - (ii) an ink layer over said protective lacquer layer; and
  - (iii) an adhesive layer over said ink layer, said adhesive layer comprising an adhesive of the type present in a water-based adhesive emulsion or in a water-based adhesive dispersion, said adhesive being the type present in an acrylic polymer emulsion having a solids content of approximately 45%, by weight, a pH of about 8.3, a weight of about 8.7 pounds/U.S. gallon, a Brookfield viscosity of about 450 cps and a glass transition temperature of about 21° C.

\* \* \* \* \*